

111

## UNITED STATES PATENT OFFICE

2,073,452

## PROCESS FOR CARROTING FUR

Warren C. Mercier, Danbury, Conn., assignor to  
American Hatters & Furriers Co., Inc., Dan-  
bury, Conn., a corporation of New York

No Drawing. Original application March 28,  
1931, Serial No. 526,131. Divided and this ap-  
plication April 14, 1934, Serial No. 720,565

2 Claims. (Cl. 8—21)

This invention relates to the art of treating fur and like fibers to give them felting properties, and to a composition of matter adapted to impart such properties to the fibers.

5 One of the objects of the invention is to provide a composition and process adapted for the manufacture of strongly adhering felt. Another object of the invention is to provide a composition and process which gives fur tight felting 10 qualities. Another object of the invention is to provide a composition and process adapted for the production of a fast-shrinking fur. Another object of the invention is to provide a composition and process adapted to produce a quick starting fur. Another object of the invention is to provide a composition and process that will not 15 discolor the fur fibers.

Another object of the invention is to provide fur or like fibers which may be immediately felted 20 after treatment according to the invention. Another object of the invention is to provide fur or like fibers which do not deteriorate materially over a long period of time. Another object of the invention is to so treat fibers adapted to the 25 production of felt that a low grade of fibers may be used, either as filler or otherwise. Another object of the invention is to achieve a thorough oxidation of a constituent substance of the fibers. Other objects will be in part obvious or in part 30 pointed out hereinafter.

The invention accordingly consists in the features of composition, combinations of elements, and in the several steps and relation and order of each of said steps to one or more of the others 35 thereof, all as will be illustratively described herein, and the scope of the application of which will be indicated in the following claims.

As conducive to a clear understanding of the several features, it may be noted that the subject 40 matter of this invention deals primarily with a composition of matter adapted to affect or modify fur or similar fibrous animal products in order that felt may be manufactured therefrom into such articles as hats, and also with the art of 45 treating such fibers to give them felting qualities. A process that imparts felting qualities to fibers is known in the art as carroting. The felting of such fibers involves the shrinking of the body which they collectively compose and a thick- 50 ening of the fibers in the sense that the finished, felted product contains a greater number of them to the square inch and the body which they compose is usually actually thicker in measurement at the completion of the felting operation 55 than it was when initially formed. Considering,

by way of example, the manufacture of a hat, the treated fibers are deposited loosely upon a cone, and, after being wet, are removed from the cone and are found to cling together and form a definite object which has certain dimensions. As a result of the felting of these fibers, by the operations known as starting and sizing, the length and breadth of the hat body are greatly reduced, while the material as a whole gains in thickness and strength. Considering the individual fibers, this felting operation involves a relative movement among them whereby, being initially spread out quite thinly, they are finally, at the completion of the operation, densely and tightly compacted together and intertwined, giving the resultant hat adequate strength to withstand ordinary usage.

The exact nature of the change wrought in a fur fiber by any particular carroting operation, whereby, under the manipulation given to a body during the felting operation it acts to produce, 20 collectively with other fibers, the transformation of the product above indicated, is in dispute, various authorities holding different theories which are not entirely in harmony with each other. 25 Although, not being certain which if any of the already advocated theories is correct, I shall not herein enter into any of them in detail, I may use certain terms which have a significance in connection with one or more of such theories, 30 but I wish it understood that my invention is not limited by any theory, being fully pointed out herein and distinctly claimed so that any one skilled in this art can understand how to practice the invention and will recognize what is reserved to me by the claims.

The usual method of applying a carroting solution is to brush it into the fur while the latter is still on the skin. In other words the fur pelts are treated with the carroting solution by the use 40 of a brush. In carrying out the process of this invention, I preferably apply the solution of the invention in this manner. The fur is then dried and thereafter may be removed from the skin and immediately made into felt.

I have found that a good carroting action can be achieved by oxidizing the fur provided the oxidizing agent used is very powerful. This application is a division of my copending application Serial No. 526,131 filed March 26, 1931, Patent No. 1,955,678. In that other application I disclosed a strong oxidizing agent as a carrot but indicated that a solution of an oxidizing agent and a hydrolyzing agent was preferred, and claimed such a solution and also the process involved in using it.

5

10

15

20

25

30

35

40

45

50

55

55

The present application deals with the use of an oxidizing agent irrespective of other action, and as an example of an oxidizing agent which has no other action I mention hydrogen peroxide.

5 Until comparatively recently, hydrogen peroxide was commercially obtainable only in comparatively weak solutions, the so-called 3 per cent solution being the standard commercial product. The 3 per cent solution corresponds approximately 10 with a solution containing 10 volumes of the oxygen gas to 1 volume of water. The active qualities of hydrogen peroxide are principally due to the fact that it liberates atomic oxygen, which is oxygen in a much more chemically reactive form 15 than the molecular oxygen such as is a constituent part of the atmosphere. The higher the concentration of this atomic oxygen in the hydrogen peroxide solution, the more atomic oxygen will be liberated, and I have found that, with respect to 20 fur fibers, increasing the strength to high concentrations results in a different action upon the fur, possibly due to the breakdown of certain constituent fur substances or molecules, which perhaps, are able to withstand an ordinary oxidizing agent, 25 such as represented by hydrogen peroxide in the weaker solutions.

Recent advances in commercial chemistry have 30 made available 100 volume hydrogen peroxide containing 100 volumes of the oxygen gas to 1 of water, and this substance is known as "Albone C." There has also recently been made available a 35 still more concentrated hydrogen peroxide containing 200 volumes of oxygen gas to 1 of water. I may use either of these substances as the strong oxidizing agent, and I may dilute either of them with water to obtain the exact desired concentration for a particular kind of fur or other fibers, or to obtain particular qualities in such fibers. Those skilled in this art will understand that owing 40 to variations between the characteristics of different kinds of fur, and owing to different manufacturing conditions and differences of temperature and humidity, it is desirable to have different strengths of solutions for different conditions.

45 As illustrative embodiments of the composition and process of the invention, I give the following preferred examples of solutions:—

|                           | Volume strength |
|---------------------------|-----------------|
| 50 1. "Albone C".....     | 50              |
| 2. "Albone C".....        | 100             |
| 3. Hydrogen peroxide..... | 200             |

55 It will be understood that other strong oxidizers of equivalent strength might be used and that the addition of substances other than acid hydrolyzing agents (claimed in my copending application) or "cleansing" agents (Parks Patents 1,507,891 and

2) is immaterial so far as this invention is concerned as the "Albone C" strong peroxide has a carotting action by and of itself. It must be further understood that I herein make no representation that 50, 100 or 200 volume hydrogen peroxide has all the qualities and effects of hydrogen peroxide in combination with a good acid hydrolyzing agent as claimed in my copending application. However I note that no discoloration of the fur is effected by use of the carotting solution of this application; a tight hat can be formed and for certain kinds of hats, provided the fur can be felted right away, it is preferable to hydrogen peroxide and mercury nitrate—nitric acid carot because the resultant fur is lighter in weight, no mercury being deposited. However, if the feel of the hat is important I recommend the carot of my copending application, and so also if expense of the carot is important. I also note that precautions should be taken to prevent the wet skin from burning after carotting when pure peroxide according to the present divisional application is used. But for certain grades of fur and for the manufacture of very light weight hats particularly for ladies' "bonnets," the matter of weight is an important consideration and the present carot will be preferred on that account. Fur treated according to the present invention of this divisional application may be dyed in the usual manner, and it is found that there is no under-cast to the fur after dyeing.

30 From the above it will be readily seen that there is herein provided a composition of matter and an art of preparing fur or similar material which attains the objects of this invention, including many distinct practical and useful advantages. Furthermore, the art of preparing the material is one which may be efficiently carried on in a practical commercial manner.

35 As various possible embodiments might be made of the above invention, and as many changes might be made in the embodiments above set forth, without departing from the scope of the invention, it is to be understood that all matter hereinbefore set forth is to be interpreted as illustrative and not in a limiting sense.

40 I claim:

1. The herein described art of preparing fur or the like for felting which consists in applying to the fibers hydrogen peroxide of a volume strength 50 between 50 and 200.

2. The herein described art of preparing fur or the like for felting which consists in applying to the fibers hydrogen peroxide of at least 100 volume strength.

55 WARREN C. MERCIER.